

# United States Patent

[11] 3,607,288

[72] Inventor **Cortland R. Burt**  
Rochester, N.Y.  
[21] Appl. No. **736,276**  
[22] Filed **June 12, 1968**  
[45] Patented **Sept. 21, 1971**  
[73] Assignee **E. I. du Pont de Nemours and Company**  
Wilmington, Del.

[56] **References Cited**  
UNITED STATES PATENTS  
3,361,564 1/1968 Bigelow et al. .... 96/101  
FOREIGN PATENTS  
723,019 2/1953 Great Britain..... 96/64

*Primary Examiner*—Norman G. Torchin  
*Assistant Examiner*—R. E. Fichter  
*Attorney*—Lynn Barratt Morris

[54] **RADIATION-SENSITIVE SILVER HALIDE  
EMULSIONS CONTAINING AMINE BORANES AND  
GOLD COMPOUNDS**  
**11 Claims, No Drawings**  
[52] U.S. Cl..... **96/101,**  
96/64  
[51] Int. Cl..... **G03c 1/36**  
[50] **Field of Search**..... 96/101, 64

**ABSTRACT:** In direct positive emulsions chemically fogged with amine boranes, the tendency for red light to bleach the image because of red light sensitivity is reduced by digesting the molten emulsion in the presence of a water-soluble gold compound. The gold compound is added in an amount from  $0.400 \times 10^{15}$  to  $3.40 \times 10^{15}$  moles of  $\text{Au}^{+++}$  or  $\text{Au}^+$  per 1.5 moles of silver nitrate. The gold compound may be added before or after the addition of the amine borane fogging agent.

RADIATION-SENSITIVE SILVER HALIDE EMULSIONS  
CONTAINING AMINE BORANES AND GOLD  
COMPOUNDS

BACKGROUND OF THE INVENTION

1. Field of the Invention

This invention relates to radiation sensitive direct-positive photographic elements. This invention also relates to radiation sensitive direct-positive silver halide emulsions for said elements. More particularly, this invention is directed to direct-positive silver halide emulsions having reduced red light sensitivity and low susceptibility to the Herschel effect.

2. Description of the Prior Art

Direct-positive elements are, of course, known and they may be imaged in a variety of ways. For example, a silver halide emulsion may be given a short overall exposure of high intensity radiation and then given a longer imagewise exposure to radiation of lower intensity. Upon development, a direct-positive image will be obtained. Another method is to expose imagewise and develop and then flash expose and redevelop. A still further method is to chemically fog the silver halide grains with, for example, formaldehyde, hydrazine, sodium arsenite, silver ions and other nonsulfide fogging agents, instead of using a solarizing exposure. Upon imagewise exposure and development of such a chemically fogged element, a positive image is obtained. In direct-positive photographic elements utilizing this latter method, there is usually incorporated a desensitizing compound, usually a colored desensitizing dye. A new direct-positive emulsion which is an improvement over the above type uses alkyl amine boranes as the fogging agents. This is disclosed and claimed in Bigelow and Burt, U.S. Pat. No. 3,361,564. This newer product gives images of high reversal density and high speed. This product does not require the use of a colored desensitizing dye and therefore the direct-positive images are free of stain which was one of the disadvantages of the prior art direct-positive elements. The use of alkyl amine boranes in silver halide emulsions eliminates the need for more than one exposure and eliminates the need to use formaldehyde as the fogging agent. Formaldehyde not only acts as a fogging agent but has a strong effect on the hardness of the colloid carrier. Although the use of alkyl amine boranes as fogging agents in direct-positive emulsions has many advantages over the prior art, it suffers from the disadvantage of being overly sensitive in the red region of the spectrum and easily bleaches upon multiple exposure through popular orange and ruby masking materials because of this red light sensitivity.

SUMMARY OF THE INVENTION

This invention relates to direct-positive emulsions and to their preparation by incorporating an amine borane compound in fogging amounts with a silver halide emulsion; and at some point prior to the end of digestion, adding from  $0.400 \times 10^5$  to  $3,400 \times 10^{15}$  mole of  $\text{Au}^{+++}$  or  $\text{Au}^+$  per 1.5 mole of silver halide of a soluble gold compound, e.g., auric chloride and aurous thiocyanate. The emulsion preferably is a gelatino-silver chlorobromide emulsion containing from about 80 to 90 percent by weight of silver bromide, the rest being silver chloride and optionally the system may contain, in addition to the two halides, from 0 to 6 percent by weight of silver iodide. The borane fogging agents may be added to the emulsion in amounts ranging from 0.0005 gram to 18.0 grams per 1.5 moles of silver halide and preferably from 0.20 to 2.00 grams per 1.5 moles of silver halide. They may be added either as a solid or dissolved in a suitable solvent. The effectiveness of the borane compounds in fogging a silver halide emulsion is influenced by the pH of the system, the higher the pH, the greater the fogging for a given amount of borane compound. Of course, certain of the borane compounds are more effective than others when used in equivalent quantities. The fogging amounts of a particular amine borane within the above limits can easily be determined empirically. The fogging effect produced by the borane compounds is bleachable by

light exposure prior to development including the red region of the spectrum. A suitable developer may be any conventional alkaline photographic developing solution which would be used for standard processing of the above direct-positive emulsions in the absence of the amine borane compounds. Among the amine borane compounds which have been found useful are those disclosed in Bigelow and Burt, U.S. Pat. No. 3,361,564 and Burt, U.S. Ser. No. 472,313 filed July 16, 1965, U.S. Pat. No. 3,445,235, May 20, 1969. For most efficient fogging action it is preferred that the amine borane compounds be added to the silver halide emulsion after it has been made, ripened, and washed to remove the excess salts resulting from the precipitation of the silver halides. Conveniently, the borane compounds are added just prior to or during the digestion or after ripening period. The pH of the emulsion is adjusted to between 5 and 9 and maintained at this level during digestion. It is at this point that the soluble gold salt is added either before, during or after the addition of the amine borane compound. As shown in example II, the gold salt can be added after the digestion step.

In addition to auric chloride and aurous thiocyanate mentioned above, other soluble gold salts may be used, e.g., sodium chloroaurate, potassium aurate, potassium chloroaurate, potassium bromaurite, potassium iodoaurite, potassium iodoaurate, potassium auricyanide and potassium aurithiocyanate. While the silver halide system used in this invention is generally of the silver chlorobromide type other types may be used such as silver chloride, silver iodobromide and silver iodochloride.

DESCRIPTION OF THE PREFERRED EMBODIMENT

While a minimum of  $0.400 \times 10^{15}$  per 1.5 moles of silver nitrate and a maximum of  $3.40 \times 10^{15}$  mole of gold ( $\text{Au}^{+++}$  or  $\text{Au}^+$ ) show good results the preferred range is from  $0.800 \times 10^{15}$  to  $3.00 \times 10^{15}$  per 1.5 moles of silver nitrate.

To test the effect of digesting the amine borane fogged emulsions in the presence of a soluble gold salt, the coated layers were sensitometrically tested using 3200° K. quartz iodine illumination. Generally the speeds and maximum densities of the samples in the example below were comparable. Typical 100/E speeds at a density of 0.25 are  $2800 \times 10^{16}$  with 4.50 maximum densities and 0.01–0.04 minimum densities. The coated elements were also exposed to the quartz iodine illumination of 960 foot-candles for 3 minutes through a Wratten 025 (Red) filter (manufactured by the Eastman Kodak Company), developed, fixed, washed, dried and read with a densitometer. The densities obtained are proportional to the resistance of the emulsion to bleaching when exposed to red light.

The invention will now be illustrated by the following example.

EXAMPLE I

To acidified aqueous solutions of gelatin each containing 1.5 moles of potassium chloride and 18 milligrams of rhodium chloride ( $\text{RhCl}_3 \cdot 3\text{H}_2\text{O}$ ) there were rapidly added solutions containing 1.5 moles of silver nitrate. To each of the resulting mixtures there was added an aqueous solution containing 0.4 mole of potassium bromide. The emulsions were ripened by heating for 10 minutes at 160° F. A second aqueous solution containing 0.6 mole of potassium bromide was added to each of the emulsions which were then ripened for 10 minutes at 160° F.

The resulting emulsions were then coagulated, washed and redispersed in the manner disclosed in Moede, U.S. Pat. No. 2,772,165 issued Nov. 27, 1956. The temperature of the redispersed emulsion was raised to 130° F. and there was then added to each 87 grams of gelatin, and the pH was adjusted to 5.7 with NaOH. Morpholine borane and trimethylamine borane were then added as indicated in the following table and the emulsions were digested at 130° F. for 40 minutes. During this period, gold salts were added in the amounts indicated in

said table. The usual coating aids including a gelatin hardener were then added and the emulsions were each coated on a polyethylene terephthalate film support having an anchoring polymer substratum and dried in the conventional manner. Sample strips of the coated films were exposed as described above and developed for 1-1/2 minutes at 60° F. in a developer having the composition:

|                                         |            |
|-----------------------------------------|------------|
| Water                                   | 750.0 ml.  |
| N-methyl-p-aminophenol hydrogen sulfate | 1.5 grams  |
| Sodium Sulfite (anhydrous)              | 19.5 grams |
| Hydroquinone                            | 6.0 grams  |
| Sodium Carbonate (anhydrous)            | 24.0 grams |
| Potassium Bromide                       | 0.8 grams  |
| Water to make                           | 1.0 liter  |

The strips were then immersed in a conventional short stop for 5 to 10 seconds and then fixed for 3 minutes in a conventional fixer, and then washed and dried. Evaluation of the resulting samples gave the following results.

| Sample No. | Mole Au <sup>+++</sup> or Au <sup>+</sup> per 1.5 moles AgNO <sub>3</sub> | Gold compd.             | Amine borane fogging agent                                      | Density after exposure to red light |
|------------|---------------------------------------------------------------------------|-------------------------|-----------------------------------------------------------------|-------------------------------------|
| 1.....     | 0                                                                         | None.....               | 3.8 mg./1.5 moles AgNO <sub>3</sub> morpholine borane.          | 1.35                                |
| 2.....     | .418×10 <sup>-5</sup>                                                     | AuCl <sub>3</sub> ..... | do.....                                                         | 2.47                                |
| 3.....     | .837×10 <sup>-5</sup>                                                     | AuCl <sub>3</sub> ..... | do.....                                                         | 3.20                                |
| 4.....     | 1.675×10 <sup>-5</sup>                                                    | AuCl <sub>3</sub> ..... | do.....                                                         | 4.50+                               |
| 5.....     | 3.350×10 <sup>-5</sup>                                                    | AuCl <sub>3</sub> ..... | do.....                                                         | 4.50+                               |
| 6.....     | 6.700×10 <sup>-5</sup>                                                    | AuCl <sub>3</sub> ..... | do.....                                                         | 4.50+                               |
| 7.....     | 13.400×10 <sup>-5</sup>                                                   | AuCl <sub>3</sub> ..... | do.....                                                         | 4.50+                               |
| 8.....     | 1.254×10 <sup>-5</sup>                                                    | AuCl <sub>3</sub> ..... | 160 mg./1.5 moles AgNO <sub>3</sub> of trimethyl amine borane.  | 4.50+                               |
| 9.....     | 2.746×10 <sup>-5</sup>                                                    | AuCl <sub>3</sub> ..... | 3.8 mg./1.5 moles AgNO <sub>3</sub> tertiary butylamine borane. | 4.50+                               |
| 10.....    | 1.875×10 <sup>-5</sup>                                                    | AuCNS.....              | 3.8 mg./1.5 moles AgNO <sub>3</sub> morpholine borane.          | 4.50+                               |

Increasing density values indicate increasing resistance to red light bleaching (1,000 watt quartz iodine lamp with Wratten 025 filter). At levels of gold compound (Samples 5, 6 and 7) above  $3.350 \times 10^{-5}$  mole Au<sup>+++</sup> there is no improvement in resistance to red light bleaching.

#### EXAMPLE II

An emulsion was made as described in example I and 3.8 milligrams of morpholine borane per 1.5 moles of silver nitrate was added as the fogging agent. After the digestion step, the gold salt, auric chloride, was added in the quantities indicated in the table below. There were then added as one of the final additions, 200 milligrams per 1.5 moles of silver nitrate of the optical sensitizing dye, 3-carboxymethyl-5[(3-ethyl-2(3-thiazolinylidene) ethylidene]rhodanine. This increased the speed of the coated element about 4-fold over that of an element not containing the dye. The resulting emulsion was coated, dried, exposed and processed as described in example I to give the following results:

| Sample No. | Mole Au <sup>+++</sup> /1.5 moles AgNO <sub>3</sub> | Density after exposure to red light 3 minutes, 960 foot-candles filtered with Wratten 025 filter |
|------------|-----------------------------------------------------|--------------------------------------------------------------------------------------------------|
| 1          | 0                                                   | 0.37                                                                                             |
| 2          | 0.837×10 <sup>-5</sup>                              | 0.87                                                                                             |
| 3          | 1.675×10 <sup>-5</sup>                              | 4.00                                                                                             |
| 4          | 3.350×10 <sup>-5</sup>                              | 4.50                                                                                             |

Increasing density values indicate increasing resistance to red light bleaching.

Other sensitizing dyes, e.g., carbocyanine and merocyanine dyes, including those described in U.S. Pat. No. 2,493,748, Jan. 10, 1950, can be used in the emulsion of this invention.

From emulsion-coated elements of the above example, good duplicates can be made by contact-printing, using either carbon arc lamps or tungsten photofloods as a light source. The emulsion-coated elements may be used for reproducing continuous tone negatives, halftones, line copy, engineering drawings, etc. The direct-positive elements of this invention may also find use in color photography.

The photographic elements of this invention provide direct positives having extremely low minimum densities and high maximum densities and are fast but at the same time show a high resistance to bleaching due to red light sensitivity. As indicated above, the elements of this invention may be developed in any conventional developing solution using standard techniques. Variations in the developer composition will have much the same effect as it would have in developing conventional nonreversal emulsions. No preexposure operations or auxiliary processing procedures are necessary or desirable in using the novel elements of this invention. It is also unnecessary to utilize stain producing desensitizing dyes or other desensitizing compounds in the emulsions. The amine boranes as chemical fogging agents are far superior to formaldehyde,

the well known and conventional fogging agent of the prior art, because the amine borane compounds do not have any hardening effect on the gelatin layer. The amine boranes have one small disadvantage and that is desensitization by kinking but this is easily overcome by the addition of a group VIII metal salt, e.g., rhodium chloride as disclosed and claimed in Burt, U.S. Ser. No. 472,313 filed July 15, 1965.

In place of gelatin, other material or synthetic water-permeable organic colloid binding agents can be used. Such agents include water-permeable or water-soluble polyvinyl alcohol and its derivatives, e.g., partially hydrolyzed polyvinyl acetates, polyvinyl ethers, and acetals containing a large

number of extralinear -CH<sub>2</sub>CHOH- groups, hydrolyzed interpolymers of vinyl acetate and unsaturated addition polymerizable compounds such as maleic anhydride, acrylic and methacrylic acid ethyl esters and styrene. Suitable colloids of the last-mentioned type are disclosed in U.S. Pat. Nos. 2,276,322; 2,276,323; and 2,397,866. The useful polyvinyl acetals include polyvinyl butyraldehyde acetal and polyvinyl sodium o-sulfonylbenzaldehyde acetal. Other useful colloid binding agents include poly-N-vinyl lactams of Bolton, U.S. Pat. No. 2,495,918, the hydrophilic copolymers of N-acrylamide alkyl betaines described in Shacklett, U.S. Pat. No. 2,833,050 and hydrophilic cellulose ethers and esters.

The emulsions of this invention may be coated on any suitable support including paper and transparent film supports. For example, the cellulose supports, e.g., cellulose acetate, cellulose triacetate, cellulose mixed esters, etc., may be used. Polymerized vinyl compounds, e.g., copolymerized vinyl acetate and vinyl chloride, polystyrene, and polymerized acrylates may also be mentioned. The film formed from the polyesters made according to the teachings of Alles, U.S. Pat. No. 2,779,684 and the patents referred to in the specification of that patent. Other suitable supports are the polyethylene terephthalate/isophthalate of British Pat. No. 766,290 and Canadian Pat. No. 562,672 and those obtainable by condensing terephthalic acid and dimethyl terephthalate with propylene glycol, diethylene glycol, tetramethylene glycol or cyclohexane-1,4-dimethanol (hexahydro-p-xylene alcohol). The films of Bauer et al., U.S. Pat. No. 3,052,543 may also be used. The above polyester films are particularly suitable

because of their dimensional stability. The emulsions are generally coated on the supports in quantities to give a coating weight of about 50-75 milligrams of silver halide per square decimeter of support surface area.

The embodiments of the invention in which an exclusive property or privilege is claimed are defined as follows:

1. A digested, radiation-sensitive direct-positive silver halide emulsion containing fogging amounts of at least one amine borane compound and at least one water-soluble gold compound in an amount to provide at least  $0.400 \times 10^{15}$  mole of  $\text{Au}^{+++}$  or  $\text{Au}^+$  per 1.5 moles of silver halide.

2. An emulsion according to claim 1 wherein the binding agent for the silver halide embodies gelatin.

3. An emulsion according to claim 1 wherein the amine borane is an alkyl amine borane of the formula:



wherein  $\text{R}_1$  is an alkyl radical of 1 to about 20 carbon atoms, and  $\text{R}_2$  and  $\text{R}_3$  are each taken from the group consisting of H and alkyl radicals of 1 to about 20 carbon atoms.

4. An emulsion according to claim 1 wherein the amine borane is trimethylamine borane.

5. An emulsion according to claim 1 wherein the amine borane is tertiarybutylamine borane.

6. An emulsion according to claim 1 wherein the amine borane is a heterocyclic amine borane.

7. An emulsion according to claim 1 wherein said amine borane is morpholine borane.

5 8. An emulsion according to claim 1 wherein said silver halide is silver chlorobromide containing 80-90 percent silver bromide.

9. An emulsion according to claim 1 containing an optical sensitizing dye.

10 10. A process which comprises admixing with a liquified radiation-sensitive silver halide emulsion prior to completion of digestion, fogging amounts of at least one amine borane compound and prior or subsequent to completion of digestion at least one water-soluble gold compound in an amount sufficient to provide  $0.400 \times 10^{15}$  to  $3.40 \times 10^{15}$  mole of  $\text{Au}^{+++}$  or  $\text{Au}^+$  per 1.5 moles of silver halide.

15 11. A process according to claim 10 wherein the emulsion is a gelatin containing emulsion and the gold compound is auric chloride.

20

25

30

35

40

45

50

55

60

65

70

75

UNITED STATES PATENT OFFICE  
CERTIFICATE OF CORRECTIONPatent No. 3,607,288 Dated September 21, 1971  
Inventor(s) Cortland R. Burt

It is certified that error appears in the above-identified patent and that said Letters Patent are hereby corrected as shown below:

In the ABSTRACT, line 6, " $0.400 \times 10^{15}$ " to  $3.40 \times 10^{15}$ " should be  $--0.400 \times 10^{-5}$  to  $3.40 \times 10^{-5}$ ...

Column 1, line 55, " $0.400 \times 10^5$ " to  $3,400 \times 10^{15}$ " should be  $--0.400 \times 10^{-5}$  to  $3.400 \times 10^{-5}$ ...

Column 2, line 33, " $0.400 \times 10^{15}$ " should be  $--0.400 \times 10^{-5}$ ;  
line 34, " $3.40 \times 10^{15}$ " should be  $--3.40 \times 10^{-5}$ ;  
lines 35 and 36, " $0.800 \times 10^{15}$ " to  $3.00 \times 10^{15}$ " should be  $--0.800 \times 10^{-5}$  to  $3.00 \times 10^{-5}$ ;

line 42, " $2800 \times 10^{-16}$ " should be  $--2800 \times 10^{-6}$ ...

Column 3, line 46, " $3.350 \times 10^{15}$ " should be  $--3.350 \times 10^{-5}$ ;  
line 72, " $0.837 \times 10^{15}$ " should be  $--0.837 \times 10^{-5}$ ;  
line 73, " $1.675 \times 10^{15}$ " should be  $--1.675 \times 10^{-5}$ ;  
line 74, " $3.350 \times 10^{15}$ " should be  $--3.350 \times 10^{-5}$ .

Column 5, line 4, " $0.400 \times 10^{15}$ " should be  $--0.400 \times 10^{-5}$ .

Column 6, line 15, " $0.400 \times 10^{15}$ " to  $3.40 \times 10^{15}$ " should be  $--0.400 \times 10^{-5}$  to  $3.40 \times 10^{-5}$ .

Signed and sealed this 16th day of May 1972.

(SEAL)

Attest:

EDWARD M.FLETCHER, JR.  
Attesting Officer

ROBERT GOTTSCHALK  
Commissioner of Patents